

F. J. METZGER,  
ELECTROLYTIC CELL,  
APPLICATION FILED OCT. 16, 1908.

1,178,591.

Patented Apr. 11, 1916.



Fig. 2



WITNESSES

*Julius Hertz*  
*D. E. Hardenburgh, Jr.*

INVENTOR  
*Floyd J. Metzger*  
BY  
*Appleton & Bruce*

ATTORNEYS.

# UNITED STATES PATENT OFFICE.

FLOYD J. METZGER, OF NEW YORK, N. Y., ASSIGNOR, BY DIRECT AND MESNE ASSIGNMENTS, OF ONE-THIRD TO HAL T. BEANS AND ONE-THIRD TO MILTON C. WHITAKER, BOTH OF NEW YORK, N. Y.

## ELECTROLYTIC CELL.

1,178,591.

Specification of Letters Patent. Patented Apr. 11, 1916.

Application filed October 16, 1908. Serial No. 458,065.

To all whom it may concern:

Be it known that I, FLOYD J. METZGER, a citizen of the United States, and a resident of New York, in the county of New York, borough of Manhattan, and State of New York, have invented a new and useful Improvement in Electrolytic Cells, of which the following is a specification.

While the invention is capable of general application in numerous situations where it is desirable to more or less separate the anode and cathode elements, I will describe the same in connection with the extraction of nickel which has been extracted from its ore and carried in a hydrochloric acid solution, but I desire it understood that the invention is in no way limited to the exact use stated and to be hereinafter described.

My invention is fully and clearly shown in the accompanying drawings wherein—

Figure 1 is a diagrammatic representation of the cell. Fig. 2 is a section of a portion of the birchwood cup showing the longitudinal position of the fibers.

1 is any suitable vessel for containing the solution.

2, 2, are carbon anodes.

3 is a nickel cathode.

4 is a cup shaped diaphragm dividing

the electrolytic cell into the anode and cathode compartments. The precise material of which I have constructed this diaphragm has been seasoned birchwood formed by milling tools into a cup, the walls of which are about one-eighth to one-quarter inch in thickness and the grain of which runs substantially in a longitudinal direction so that at the sides of the cup the side of grain is presented to the electrolyte and at the bottom the end of the grain is presented thereto. In some cases, I have prepared this cup for use by soaking it in alcohol to remove resinous substances and in others not. It is the purpose of this wood diaphragm to prevent diffusion of any of the products resulting from electrolysis, which products, if allowed to circulate freely in a solution without a diaphragm, would enter into chemical combination and defeat the object

of the electrolyzation. For instance, in the experiment described in this application in which nickel is the metal to be recovered,

chlorin must be kept away from the deposited nickel.

In carrying out my invention, I have proceeded as follows by way of example: I have treated water solutions of nickel chlorid of about 1.3 specific gravity obtained by subjecting nickel ore to hydrochloric acid. During the reaction stated in the above example, ionized chlorin migrates through the diaphragm 4 toward the anode where it is changed to chlorin gas, part of which is evolved as such, and part remains dissolved in the electrolyte. The diaphragm described prevents this chlorin dissolved in the electrolyte as well as the chlorin gas from diffusing and reentering the cathode chamber and attacking the deposited metal.

The use of the separating diaphragm consisting of a wood or fibrous body in which the grain of the wood, or the fibers of the body are arranged endwise to the adjoining solution, constitutes the important feature of my invention for the following reasons: By the use of a diaphragm in which the wood is cut cross-grain there is practically no resistance to the current even though the diaphragm is of considerable thickness, say, from one-quarter to one-half an inch, and in consequence of this I am able to secure a very high current efficiency during the progress of the process. As will be seen from the example hereinafter set forth, the current efficiency is nearly 100 per cent. A further advantage of the diaphragm cut cross-grain or in which the fibers lie endwise to the solution, resides in the fact that the electrolyte can pass through the diaphragm, but none of the gases evolved in the reaction which takes place are permitted to do so. I do not desire to be limited to any particular kind of wood and have mentioned birchwood above as being one of the woods which I have used successfully in carrying out the process. Having placed said nickel chlorid solution in the cell so as to occupy both the anode and cathode compartments the time, current and temperature of the operation may be exemplified by the following tabulation of a specific case in which I obtained a deposit on the cathode 3 of about 33 grams of nickel in about 3 hours with a current of from 10 to  $10\frac{1}{2}$  amperes and about 4½ volts;

the cathode surface being about 15 square inches and there being no apparent depreciation in the efficiency of the diaphragm.

| 5  | Hour of observation. | Amperes. | Volts. | Temperature, centigrade. |
|----|----------------------|----------|--------|--------------------------|
|    | 2.25                 | 10.2     | 4.6    | 78                       |
|    | 3.15.                | 10       | 4.8    | 72                       |
|    | 3.45.                | 10.2     | 4.5    | 78                       |
|    | 4.35.                | 10.3     | 4.4    | 78                       |
| 19 | 5.20.                | 10.5     | 4.5    | 72                       |
|    | 5.35.                | 10.5     | 4.5    | 72                       |

I have above described the manner in which I have practised my invention with 15 great particularity and exactness so as to make it absolutely certain, that a person following the description will obtain the same result, but I do not therefore wish to be understood as implying that all of these 20 details are necessary or limit myself to them since I believe that they may be departed from. For example, if, in the light of this description, it shall be found that other kinds of fiber, whether wood or other vegetable fiber, can be substituted for the birch-wood, I will consider the same to be within 25 the scope of my invention. I also know from my own experiments that in many respects the above described details may be departed from more or less; for example, by 30 properly increasing the amount of current no external heat is necessary to maintain the bath at the proper temperature.

I should also point out that in the precise 35 form of my invention shown the bottom of the cup shaped diaphragm 4 is raised above the bottom of the cell and above the lower

ends of the anodes so that the solution in the anode compartment extends across between the anodes beneath the bottom of the cup. 40

Having thus described my invention, what I claim is:

1. In an electrolytic cell, the combination of an anode, a cathode and a diaphragm extending across substantially the entire effective path of the current to and from said electrodes, said diaphragm being formed of fibrous material having the ends of the fibers presented to the electrolyte. 45

2. In an electrolytic cell, the combination of an anode, a cathode and a diaphragm extending across substantially the entire effective path of the current to and from said electrodes, said diaphragm being formed of wood with the ends of the grains presented 55 to the electrolyte. 50

3. A diaphragm for an electrolytic cell comprising a section of fibrous material formed to present the ends of the fibers to the electrolyte. 60

4. A diaphragm for an electrolytic cell comprising a piece of wood cut to present the ends of the grains to the electrolyte. 65

5. A diaphragm for an electrolytic cell comprising a piece of birchwood cut to present the ends of the grains to the electrolyte. 65

In testimony whereof I have hereunto signed my name in the presence of two subscribing witnesses.

FLOYD J. METZGER.

Witnesses:

K. G. LEARD,  
T. E. HARDENBERGH, Jr.

Copies of this patent may be obtained for five cents each, by addressing the "Commissioner of Patents, Washington, D. C."